

## UNITED STATES PATENT OFFICE.

JAMES MCINTOSH, OF NORRISTOWN, PENNSYLVANIA, ASSIGNOR TO DIAMOND STATE FIBRE COMPANY, OF BRIDGEPORT, PENNSYLVANIA, A CORPORATION OF DELAWARE.

## VENEER AND METHOD OF MANUFACTURING.

No Drawing.

Application filed May 14, 1926. Serial No. 109,179.

This invention relates to improvements in veneer strips made of paper or fabric impregnated with a phenolic or other resin of the class which is transformed under pressure and elevated temperatures to a hard, insoluble, and infusible condition.

The invention further relates to improvements in the methods of manufacturing these veneer strips.

10 Prior to my invention it had been difficult, if not impossible, to produce satisfactory veneer of the above stated type. It was difficult, for example, to produce the thin strips with a uniform high finish due to unavoidable irregularities or lack of parallelism in the plates of the press in which the veneer was manufactured. Also the under sides of the veneer strips as previously manufactured were so smooth and impervious to 15 glue or other adhesive that effective adherence of the strip to the base surfaces could not be obtained.

It is the principal objects of the present invention to overcome these defects and to 20 provide a veneer of the stated type which shall be entirely practicable.

In practicing my invention, I may employ as a base material a laminated paper board such as made on a cylinder machine. 25 Preferably the paper stock from which the board is made is short and well beaten so that the cohesion between the respective laminations is at a minimum. Or I may employ a base-board built up of a number of 30 sheets of paper so united that there is little or no coherence between the sheets. Although it is practicable to practice the invention by using a base body consisting of a mere disunited stack of paper sheets, I prefer to employ a laminated built-up board 35 of the type first mentioned.

Against one or both sides of this board or 40 stack, I place one or a number of sheets of paper or other suitable fibrous material impregnated with a synthetic or other resin of the stated type, and the resulting pile is then pressed between plates in a suitable 45 press in the usual manner of treating such materials in order to transform the resin to its final hard condition. It will, of course, 50 be understood that any suitable method of impregnating the sheets with the resin may

be employed, this operation being well understood in the art.

After the application of pressure and heat, 55 the resin-impregnated sheets will have been found to adhere to the faces of the base-board or to the outer sheets of the unimpregnated stack, and in either event the impregnated sheets in which the gum is in its 60 hard final condition may be stripped off the board or separated from the stack, with the result that a veneer sheet is provided which may be very thin yet nevertheless possesses a high uniform finish on one side and a papery 65 absorbent finish on the other side suitable for gluing, this paper finish being obtained by reason of the adherence to the face of the impregnated sheet of some of the paper base.

It will be noted that although the presses 70 may not be sufficiently accurate to insure a uniformly high finish on all parts of the veneer strips when these strips are compressed alone and without the base-board or other filling, by reason of their thinness which 75 may, for example, be .005", the base-board compensates for the irregularities in the press to such an extent that the variations are automatically taken care of, the base-board or stack acting as a cushion compensating for all unevenness in the plate and affording approximately uniform pressure 80 over the entire surface of the impregnated sheets.

Although it is preferred to employ a base-board of laminated and easily delaminated construction, since this provides simple means for affording the aforesaid papery 85 finish of a substantially uniform thickness, it will be apparent that any type of board of a suitable fibrous or absorbent material, so constructed that a part thereof will adhere to the veneer strips when the latter are removed, will suffice and there is to be no limitation in this respect.

In practice, the veneer strips adhering to one or both faces of the base-board may be stored or shipped without danger of breakage, and may be stripped from the boards as required. Or they may be stripped immediately from the boards and sold or shipped in 100 condition for use. In any event a veneer is provided having all the required characteristics of a completely practicable article.

The veneer strips may be grained to imitate wood veneer, and may be given any desired finish, either highly polished or matte. Where the graining is marked on the paper sheets prior to their impregnation, the markings are in effect inlaid in the veneer and accordingly are very durable.

I claim:

1. A thin veneer sheet impregnated with a hardened resin, and fibres embedded in the resin and exposed on one face of the sheet to form an integral fibrous surface.
2. A thin veneer sheet impregnated with a hardened resin and having on one face a substantially uniform high finish, and fibres cemented by said resin to the other face of the sheet and forming an integral fibrous surface.
3. The method of manufacturing thin veneer sheets, which consists in treating a fibre sheet with a resinous binder, laying said sheet against a face of a relatively thick body of fibrous material, hardening the binder under conditions such that at least a portion of said fibrous body adheres to the face of the sheet, and thereafter removing the sheet from said body with an adhering portion of the latter forming on one face of the sheet a fibrous surface.
4. The method of manufacturing thin veneer sheets, which consists in taking a fibre sheet, impregnating said sheet with a synthetic resin in its soluble and fusible state, applying said impregnated sheet to a relatively thick body of fibrous material, applying pressure and heat to convert the resin to its final hard and infusible state, and separating the sheet from the said fibre body

with an adhering portion of the latter forming on one face of the sheet a fibrous surface.

5. The method of manufacturing thin veneer sheets, which consists in impregnating a fibre sheet with a synthetic resin in its soluble and fusible condition, applying the impregnated sheet to the face of a laminated and easily delaminated fibre body, converting the resin to its hard and infusible state under conditions such that the said laminated body adheres to the face of the sheet, and separating the sheet from the body with an adhering portion of the latter forming on one face of the sheet a fibrous surface.

6. In the manufacture of thin veneer sheets, the method of obtaining a substantially uniform high finish on the finished product, which consists in treating a fibre sheet with a resin adapted to be hardened by the application of heat and pressure, laying the treated sheet against a relatively thick and resilient body, and applying heat and pressure to harden the resin.

7. As a new article of manufacture, a body of fibrous material united to form a readily disintegrated board, said board having on one face thereof a relatively thin sheet impregnated with a hardened resin, said impregnated sheet being secured to the said board by means of the resin with which it is impregnated and by reason of the physical characteristics of said board being readily detachable therefrom, with an adhering portion of the board forming on one face of the sheet a fibrous surface.

JAMES McINTOSH.